

## UNITED STATES PATENT OFFICE

2,246,554

## BUFFING COMPOUND

Robert V. Twynning, Grand Rapids, Mich., assignor  
to J. C. Miller Company, Grand Rapids, Mich.,  
a corporation of Michigan

No Drawing. Application February 27, 1939,  
Serial No. 258,734

5 Claims. (Cl. 51—305)

This invention relates to buffing compounds such as are used in practice upon the outer surfaces of fabric buffing and polishing wheels. Such buffing compounds include essentially an abrasive and a binder therefor. Heretofore in order to get suitable properties and qualities for the binder it has been common to use several ingredients, ranging many times as high as six ingredients, though the average composition has had three or four of such ingredients. The melting temperature of the binder is one factor which must be taken into consideration, the easy removal or cleaning of the buffing composition from the surface of the buffed work is another important factor. And of course commercially an important and controlling factor is the cost of materials.

My invention is directed to the production of a buffing compound wherein the binder is a single ingredient, the preferable binding material being the residue produced and derived from hydrogenation and distillation of animal and vegetable fats by which is obtained stearic acid and other elements or compounds present in such fats. The residue left is known as stearin pitch, which is a very dark and in many cases black residue left in the stills after the volatile organic acids and glycerides have been removed. The distillation is made at a high temperature with the use of dry super-heated steam, but the residue which heretofore in many cases has been largely a waste product, though meltable at a temperature less than the temperature of the super-heated steam used, does not evaporate and volatize as do the stearic acid and glycerides.

The stearin pitch which I have found most suitable for the binder and buffing compounds, in its composition has a total of 73% fatty acids of which 14.6% are free fatty acids. The unsaponifiable material varies between 5 and 10% though I have had samples of the stearin pitch thus derived from hydrogenation and distillation of animal fats wherein the unsaponifiable content was less than 2%. The very high amount of saponifiable material is of value in the operation of cleaning or removing from the fabric of the buffing wheels, using an alkaline cleaning solution, which combines with the saponifiable material to produce soap which is not only easily washed away but itself is a cleanser.

The melting point of the stearin pitch thus produced is relatively high and the most melting point preferred is approximately 81 or 82° C. Such melting point is higher than in binders normally used for buffing compositions, in fact it is

approximately twice the temperature of melting of the present binders. Such high melting point greatly increases the efficiency of the buffing composition and helps against wear on the buffing wheel. The face of the wheel to which the buffing composition is applied is harder and firmer and is plastic, considerably reducing buffing wear by protecting the fabric and greatly reducing or eliminating "threading" of the buffing fabric.

10. The cost of the stearin pitch binder is approximately one-third the cost of present binders intended for the same purpose. With the binder there may be readily mixed the usual abrasive or buffing materials. Tripolis in finely ground or divided state may be thoroughly mixed with the stearin pitch binder when it is in melted form. It is one property or result of this binding material that the buffing composition of the stearin pitch binder and tripolis applied to a buffing wheel is free from the undesirable result of "burning" die castings even under excessive pressures, this being a marked improvement over most of the present binders.

15. The stearin pitch binder is also applicable to all buffing compositions. It can be used as the sole binder and it can also be added to binders including several ingredients, and dependent upon the quantity of stearin pitch used which may vary between 15% to 100% of the entire binder, the melting temperature may be regulated between somewhat above the low melting temperatures of present binders and the high melting temperatures, approximately twice as much, of the stearin pitch. This is of importance in many cases in connection with different materials which are to be buffed and polished and which may be best polished with a binder which is meltable at a particular and specific temperature.

20. The buffing composition which I have made, when the binder consists solely of the stearin pitch, will vary between ratios of abrasive to binder of approximately 1.8 parts of abrasive to one of binder as the minimum, and increasing with certain binders to as high as six parts of abrasive to one of binder, particularly where the abrasive, for example aluminum oxide, has very little or no properties of absorption of the binder. Tripoli rock or stone which is very much used

25. may range as to quantity between 1.8 parts to 4.5 parts for one part of the binder. While stearin pitch as the residue left or derived from hydrogenation or distillation of animal fats is preferred for the binder, the pitch residue left from the treatment to remove the essential fatty acids

from cotton seed oil or other vegetable oils is also available, particularly when mixed with the stearin pitch derived from animal fats. The term "stearin pitch" is also to be considered as inclusive of marine pitch, derived from fish oil, and various other pitches which are derived from animal or vegetable fats. But the residue left from the distillation of mineral oils, for example asphaltum pitch or from crude oil distillation are of no utility and have no application herein.

Stearin pitch as a binder may also be used for a composition for polishing wheels, in which the composition contains greases and oils rather than abrasive material. With my invention as high as 80% of the composition may consist of stearin pitch, the remaining 20% being greases or oils which are intermingled with and held together by the pitch, and the composition will have strength and rigidity so that it can be formed into suitable sticks to be pressed against the polishing wheel and adhere thereto. The binder, stearin pitch, may be reduced below 80% and in some cases as low as 40% of the total composition. But in the event that the pitch used is very greatly reduced or if it is reduced below 40%, the solidity and rigidity which the pitch gives to the composition must be helped by the use of stearic acid, with consequent greater cost. But my invention contemplates the production of buffing or polishing compounds through the utilization of stearin pitch, either as the sole binding ingredient or the use thereof in varying quantities with other well-known ingredients now commonly used for binders.

Having thus fully described my invention, what I claim and desire to secure by Letters Patent is:

1. A buffing compound comprising finely divided abrasive material and a binder therefor of stearin pitch, said pitch being the residue remaining after the hydrogenation and distillation of animal or vegetable fats to remove stearic acid and glycerides.
- 10 2. A buffing compound comprising finely divided abrasive material and a stearin pitch binder which has more than 90% thereof saponifiable.
- 15 3. A buffing compound comprising a finely divided abrasive material adapted for buffing and polishing operations upon metal or the like, and a binder therefor solid at temperatures well above atmospheric temperatures, said binder including stearin pitch produced as a residue remaining after the hydrogenation and distillation of animal fats or vegetable oils, as specified.
- 20 4. A compound of the class described comprising, a binder of stearin pitch and metal buffing or polishing material incorporated with and bound together by said pitch.
- 25 5. A compound of the class described comprising, finely divided abrasive material with stearin pitch as a binder and greases and oils disseminated therethrough and bound together thereby, for the purposes described.

ROBERT V. TWYNING.